

(No Model.)

E. MANSFIELD.

METHOD OF MAKING FERRULES FOR CANT HOOKS.

No. 442,813.

Patented Dec. 16. 1890.



Fig. 1.



Fig. 2.



Fig. 3.



Fig. 4.



Fig. 5.



Fig. 6.



Fig. 7.



Fig. 8.

Witnesses.

Irving H. Gay.  
Geo. W. White.

Inventor. Edward Mansfield  
by Alvan Andrew, his atty.

# UNITED STATES PATENT OFFICE.

EDWARD MANSFIELD, OF ORONO, MAINE.

## METHOD OF MAKING FERRULES FOR CANT-HOOKS.

SPECIFICATION forming part of Letters Patent No. 442,813, dated December 16, 1890.

Application filed September 22, 1890. Serial No. 365,725. (No model.)

To all whom it may concern:

Be it known that I, EDWARD MANSFIELD, a citizen of the United States, and a resident of Orono, in the county of Penobscot and 5 State of Maine, have invented new and useful Improvements in the Method of Making Ferrules for Cant-Hooks, of which the following, taken in connection with the accompanying drawings, is a specification.

This invention relates to improvements on the patent granted to me January 31, 1888, No. 377,038, for a method of making ferrules for cant-hooks, and it is carried out as follows, reference being had to the accompanying 15 drawings, wherein—

Figure 1 represents a plan view of the metal plate from which the ferrule is made. Fig. 2 represents a perspective view of the blank from which the staple is formed. Fig. 3 represents such staple-blank temporarily attached to the ferrule-plate previous to and during the operation of welding such parts together. Fig. 4 represents a cross-section on the line X X, shown in Fig. 3. Fig. 5 represents a sectional view showing the punch and die for welding the ferrule-plate and staple together. Fig. 6 represents a sectional view showing said ferrule-plate and staple after being welded together. Fig. 7 represents a perspective view of the ferrule after 25 being closed and welded together, and Fig. 8 represents a central longitudinal section of the finished ferrule with its wooden handle and the cant-hook pivoted to the staple of 30 said ferrule.

Similar letters refer to similar parts wherever they occur on the different parts of the drawings.

In carrying out my invention I proceed as follows: I first cut or punch out from weld- 40 steel or suitable forged or wrought metal a plate or ferrule-blank *a*, through which I make slotted perforation *a'*, as shown in Fig. 1. *b* in Fig. 2 is the staple-blank, which is also 45 preferably made from weld-steel, and provided with a vertical slit *b'*, which latter may be made, preferably, by means of a saw while the blank is heated. Said slotted staple-blank is then temporarily secured to the perforated

portion of the ferrule-blank *a*, preferably by 50 means of a metal wedge *c*, (shown in Figs. 3 and 4,) for the purpose of holding the staple-blank *b* in its proper position on the plate *a* during the process of heating and welding together said parts. After the staple-blank 55 *b* and the plate *a* have been heated to a welding heat I place the plate *a* on top of a die-block *d*, Fig. 5, having a recess *d'* corresponding to the exterior form and size to be given to the staple and having a perforation *d''*, 60 adapted to receive the punch *e*, which is of a size and form equal to the opening desired to receive the eye of the cant-hook. The punch *e* is attached to or forms a part of a plunger *e'*, as is common in drop forging or welding 65 machines. During this welding operation the plate *a* is placed upon the die-block *d*, with the staple-blank *b* projecting upward, as shown in Fig. 5. During the descent of the plunger *e'* the punch *e* enters the slit in the 70 staple-blank and passes into the die-block perforation *d''*, and as the plunger *e'* continues to descend it causes the staple-blank to be forced into the recess *d'* on the opposite 75 side of the plate *a*, leaving the now molded and welded staple projections on the outside of the ferrule-blank, as represented in Fig. 6. The advantage of this method over the one described in my above-mentioned patent is that the staple is more firmly welded to the 80 plate *a*, causing a part of the staple to be lapped over or expanded on the inside of the plate *a* in the form of lips or flanges *b'' b''*, (shown in Fig. 6,) by which an increased welding-surface is obtained between the parts, and 85 consequent increase of the strength at the welded joint. I also obtain a more even and finished appearance of the staple where it joins the exterior of the ferrule. After such parts are welded together I repeat them and 90 bend the plate *a* around a conical mandrel *f* (shown in dotted lines in Fig. 7) and weld the overlapping edges of said ferrule at *a'*, as shown in Fig. 7. The ferrule is now finished, and I drill or punch a hole through the staple 95 *b* for the reception of the bolt or rivet *g*, to which the eye *h'* of the cant-hook *h* is pivoted, as shown in Fig. 8.

*i* is the wooden rod the end of which is driven into the ferrule, as is usual in devices of this kind.

What I wish to secure by Letters Patent, 5 and claim, is—

The herein-described method of making cant-hook ferrules, consisting in first cutting or punching out a plate *a* and making a slit or perforation *a'* therein, then attaching a slotted 10 staple-blank to the inside of said ferrule-plate, welding said parts together and forcing the staple during the welding operation to the opposite side or outside of the ferrule-plate,

and finally bending the latter in the form of a conical tube and welding its abutting or overlapping edges together, substantially as and for the purpose set forth. 15

In testimony whereof I have signed my name to this specification, in the presence of two subscribing witnesses, on this 12th day 20 of September, A. D. 1890.

EDWARD MANSFIELD.

Witnesses:

ALBAN ANDRÉN,  
JULIA RICHARDSON.